

I. E. LESTER.  
CASTING OF IRON.  
APPLICATION FILED JULY 5, 1913.

1,093,443.

Patented Apr. 14, 1914.

2 SHEETS—SHEET 1.



Fig. 1



Fig. 2

WITNESSES

W. C. Baker, Jr.  
G. L. Rollman

INVENTOR

ISAAC ENOCH LESTER  
BY *M. M. Co.*  
ATTORNEYS

I. E. LESTER.  
CASTING OF IRON.  
APPLICATION FILED JULY 5, 1913.

1,093,443.

Patented Apr. 14, 1914.

2 SHEETS-SHEET 2.



Fig. 3



Fig. 4

WITNESSES

W. C. Baker, Jr.  
G. D. Rollhans

INVENTOR  
ISAAC ENOCH LESTER  
BY Minn Co  
ATTORNEYS

# UNITED STATES PATENT OFFICE.

ISAAC ENOCH LESTER, OF BIRMINGHAM, ENGLAND.

## CASTING OF IRON.

1,093,443.

Specification of Letters Patent. Patented Apr. 14, 1914.

Application filed July 5, 1913. Serial No. 777,505.

*To all whom it may concern:*

Be it known that I, ISAAC ENOCH LESTER, subject of the King of Great Britain, residing at 44 Sandwell road, Handsworth, in the city of Birmingham, England, have invented certain new and useful Improvements Relating to the Casting of Iron, of which the following is a specification.

This invention relates to the production 10 of rolls and other iron castings in which a hard surface is required together with toughness in the body or mass of the article to resist heavy loads or stresses.

As is well known a chilled roll, or other 15 casting produced in a chill or iron mold, possesses great surface hardness but is wanting in toughness, whereas a grain roll, or other casting produced in a sand mold, has a degree of toughness but lacks the surface 20 hardness of the chilled roll. It is also known that by expediting the cooling of the metal after casting in a sand mold, a certain chilling or hardening effect may be obtained.

The object of this invention is to provide 25 simple and reliable means for imparting a hard surface to an iron casting for the resistance of wear, while retaining that toughness in the body of the casting which is necessary for the resistance of stresses liable to 30 cause fracture or breakage.

The invention consists in the combination with a sand matrix, of a metal portion or heat conducting medium which is shaped and arranged to provide between it and the 35 casting a layer of sand of uniform thickness and of the same character as the sand in the remainder of the mold.

Referring to the two accompanying sheets of explanatory drawings:—Figure 1 is a diagrammatic sectional side elevation and Fig. 2 a sectional plan of a mold adapted for the production of a roll, in accordance with this invention, for the rolling of iron and steel or other metal. Fig. 3 is a diagrammatic 45 section illustrating the production of an engine cylinder in accordance with this invention, and Fig. 4 illustrates the production of another form of roll.

The same reference letters in the different 50 views indicate the same or similar parts.

In the application of the invention in connection with the production of iron rolls as shown in Figs. 1 and 2, the mold is produced in the ordinary way, but embedded therein 55 adjacent to the parts at which a hard wearing surface is required in the casting are a

number of metal segments *a* which are grouped or arranged together in any convenient manner. The inner ends or portions of the segments are shaped to correspond with the configuration of the portion of the casting to be chilled or hardened, and such portions are covered with a relatively thin coating *b* of sand of uniform thickness. Thus there is obtained a complete matrix of sand with an embedded metal portion which when the molten metal is poured into the mold produces cooling of the casting adjacent to the embedded metal at the rate necessary to give the desired qualities of hardness and toughness. By varying the thickness of the sand covering the metal portion the relative amounts of hardness and toughness can be varied to meet any particular requirement. Further, the size of the metal portion 75 may also be varied for a like purpose.

The inner ends of the metal or cooling segments are varied in shape to suit the particular section of the roll to be cast. Fig. 4 illustrates the production of a roll of different section from that shown at Fig. 1. It will be understood that the metal portion or portions are adapted to coincide with the parts of the casting where hardening is desired to be produced; the remainder of the 80 mold is of ordinary sand construction. For some purposes the whole of the mold may be constructed from metal portions having a relatively thin and uniform face of sand. Or there may be combined an ordinary chill 85 mold with any of the herein described forms of molds when a portion only of the casting is required to be of the quality produced by the application of this invention, while the remainder is to be as an ordinary chilled or 90 grained casting. Further, it will be understood that in the production of hollow castings in which the inner surface or a portion of the inner surface is desired to be hardened, the metal portions are arranged with 95 the core of the mold. Thus, in the production of an engine cylinder in which a hard inner surface is required, the core is formed from a metal block *a* having a covering *b* of sand of the required thickness as shown at 100 Fig. 3. The core may be made hollow as shown.

Having thus described my invention what I claim as new and desire to secure by Letters Patent is:—

1. In the casting of iron, the combination 110 consisting of a metal chill mold, and a thin

layer of sand of uniform thickness on the surface thereof, adapted to contact with the casting, as set forth.

2. In the casting of iron, the combination consisting of metal segments forming a chill mold, and a thin layer of sand of uniform thickness on the surface thereof, adapted to contact with the casting, as set forth.

In testimony whereof I have signed my name to this specification in the presence of 10 two subscribing witnesses.

ISAAC ENOCH LESTER.

Witnesses:

JOHN MORGAN,  
FRANCIS MALPAS.

Copies of this patent may be obtained for five cents each, by addressing the "Commissioner of Patents, Washington, D. C."